

[54] REUSABLE MANDREL FOR STRUCTURES  
HAVING ZERO DRAFT OR RE-ENTRANT  
GEOMETRIES

[75] Inventors: **Robert J. Baird**, Indianapolis, Ind.;  
**Thomas G. Everett, Jr.**, Flanders,  
N.J.

[73] Assignee: **Union Carbide Corporation**, New  
York, N.Y.

[22] Filed: **Oct. 27, 1972**

[21] Appl. No.: **301,495**

**Related U.S. Application Data**

[62] Division of Ser. No. 156,191, June 24, 1971, Pat. No.  
3,717,914.

[52] U.S. Cl. .... **117/71 M, 117/49, 117/50,**  
117/51

[51] Int. Cl. .... **C23c 1/06, C23c 1/10**

[58] Field of Search..... **117/71 M, 50, 51; 164/46,**  
164/132; 29/195 P, 191; 249/62

[56] **References Cited**

UNITED STATES PATENTS

3,717,914 2/1973 Baird et al. .... 29/195

Primary Examiner—Thomas J. Herbert Jr  
Attorney, Agent, or Firm—Dominic J. Terminello

[57] **ABSTRACT**

A mandrel, and process therefor, consisting of a high melting temperature base material, such as aluminum, having an undercoating of a low melting temperature metallic alloy and an overcoating of a polyimide material. In casting or plasma deposition applications, the undercoated metallic alloy is removed at an elevated temperature thereby facilitating the removal of the base mandrel.

7 Claims, 1 Drawing Figure



PATENTED FEB 4 1975

3,864,150



## REUSABLE MANDREL FOR STRUCTURES HAVING ZERO DRAFT OR RE-ENTRANT GEOMETRIES

This is a division of application Ser. No. 156,191 filed June 24, 1971, now U.S. Pat. No. 3,717,914.

### FIELD OF THE INVENTION

This invention relates to reusable mandrels, and the process therefor, for use in producing plasma-deposited consolidated bodies or castings having zero degree draft or reentrant geometries. Specifically, the mandrel consists essentially of a high-melting-point base mandrel, such as aluminum, having a low-melting-point metallic alloy undercoat and a polyimide overcoat.

### DESCRIPTION OF PRIOR ART

Cast structures and component parts having various complex configurations are presently being fabricated with the aid of mandrels. Simple hollow configurations having a draft or taper angle of at least 2° can be easily cast with removable and reusable mandrels. However, the fabrication of complex configurations having zero draft or re-entrant geometries presents a problem to the casting industry. Multisegmented mandrels, which can be removed in pieces after a particular structure is cast, have been employed with some success in certain applications. A drawback to this technique, however, is that a misalignment of any of the segments of the mandrel during casting will be reflected in the fabrication of a distorted structure.

Another technique employed by the casting industry is to prepare low-melting-point mandrels for use in the fabrication of high-melting-point structures. The cast unit, upon completion can be heated to a temperature below that of the structure but above that of the mandrel so that the latter can be removed in the liquid phase. This type mandrel in addition to having the disadvantage of being non-reusable, is also limited to casting applications that do not exceed the melting point of the mandrel and to the casting of only high-melting-point structures.

Recently mandrels have been successfully employed in the fabrication of plasma consolidated free-standing shapes having draft or taper angles sufficient to allow removal of the mandrels without effecting such shapes. However, mandrels can not be successfully used when the desired plasma-consolidated shapes have either zero draft or re-entrant geometries. Thus, this limitation of mandrel usage to the fabrication of relatively simple tapered shapes has forced industry to resort to complex and costly techniques to produce shapes or structures having zero draft angles or re-entrant geometries.

The primary purpose of this invention is to overcome the limitation inherent in conventional type mandrels by providing a new removable type mandrel that will be admirably suited for use in the casting and plasma-deposition of various structures having as low as zero draft or re-entrant geometries.

### SUMMARY OF THE INVENTION

Broadly stated, this invention relates to a mandreling technique admirably suited for the production of various shaped structures. Specifically, a mandrel is composed by coating a low-melting-point metallic alloy on

a high-melting-point base mandrel and then overcoating the alloy with a polyimide layer. The undercoated alloy layer has to be sufficiently thick so that after a structure is coated or sprayed onto or into the mandrel, the assembly can be heated to the melting point of the alloy so that it can be removed in the liquid state leaving a space between the structure and the mandrel sufficient to allow the mandrel to be easily removed.

The base mandrel can be cast or otherwise fabricated using a high-melting-point material selected from at least one of the groups consisting of aluminum, brass, steel, and copper. The material selected in addition to having a melting point higher than that of the metallic alloy to be coated thereon, shall be sufficiently strong so as to be reusable and should also be substantially non-reactive with the particular alloy coating selected. Likewise, the metallic alloy coating should have a low-melting point with reference to the base mandrel, and also with reference to the structure to be cast or plasma deposited. The thickness of this metallic alloy coating is variable and depends on the configuration, material and size of the structure being cast. Generally a thickness between about 1/16 inch and about 1 inch is sufficient with a thickness about 1/8 inch being preferable for general applications. Metallic alloys having a melting point below 300°C. are generally suitable for this application. However, the selected base mandrel material and structure material dictate the limitations on the characteristics required of this metallic alloy coating. Metallic alloys such as bismuth, lead, tin, cadmium, indium, and antimony in any and all proportions are suitable for use in this invention.

The primary purpose for applying an overcoat on the alloy layer is to substantially eliminate any reaction between the structure to be cast or plasma deposited and the alloy layer. Therefore this overcoating need only be applied to the portion of the coated mandrel that the structure will contact. In addition to preventing any reaction, this outer layer must have a higher melting point than the alloy, be easily separable from the cast or plasma deposited structure and be non-reactive with the deposited structure. The exact thickness of this outer coating is not critical but a layer of between about 0.002 inch and about 0.010 inch is deemed sufficient for most applications. Polyimide coatings are admirably suited for this overcoat layer. Polyimides are a relatively recently developed type of polymer with especially good resistance to heat deterioration. A typical example of a polyimide is that derived from pyromellitic dianhydride and an aromatic diamine and having the following basic structure unit:  $[-(CO)_2C_6H_2(CO)_2NC_6H_4OC_6H_4-]_n$ . The actual polymer, however, has a more complex structure due to cross linking.

The preferred method for implementing this invention is to initially fabricate a base mandrel from a high-melting-point material such as aluminum. The contour of a male or female type mandrel, in addition to substantially conforming to the configuration of the desired structure, has to be produced with radial dimensions smaller or larger, respectively, than the structure so as to allow for a dual coating buildup. Usually a 1/4 to 1/2 inch dimension discrepancy is adequate for this purpose.

An alloy having a melting point below about 700°C., preferably about 250°C., is then deposited on the mandrel by any conventional technique such as by spraying,

brushing, casting, painting or the like. The thickness of this coated layer is somewhat variable and depends primarily on the complexity of the structure desired, that is, the draft angle or any other re-entrant geometries such structure has. The purpose of this layer is to provide a certain dimensional buildup on the mandrel which can then be easily removed in a liquid state at an elevated temperature after the desired structure is cast or plasmadeposited thereon. The space created between the mandrel and the structure by such alloy removal, will then be sufficient to allow the mandrel to be manipulated and then easily removed thereby leaving a free standing body. A metallic alloy layer of between about  $1/16$  inch and about 1 inch is usually sufficient for most complex structures.

To provide good securement of the metallic alloy to the base mandrel, at least one locking type groove or projection may be designed into the base mandrel so as to prevent the base mandrel from sliding out of, or otherwise being removed from, the coated metallic alloy layer prior to the latter being removed in the liquid state. When this securement means is employed, the metallic alloy layer will usually require a machining operation to conform its surface to the contour of the desired structure to be produced. Thus, complex curvilinear structures can be fabricated using this mandreling technique.

Although this simple alloy coating would suffice in some applications, an interaction generally occurs between this low melting alloy coating and the deposited structure thereby greatly limiting its utility. To prevent this detrimental interaction, an outer layer of a neutral type plastic composition, having a curing temperature below the melting temperature of the alloy coating, is deposited by any conventional technique on the metallic alloy layer. This outer layer need only be applied to that portion of the metallic coated mandrel that will be contacted by the structure to be cast or plasma-sprayed thereon. This outer coating need only be between about 0.002 inch and about 0.010 inch thick, and be capable of being easily removed from the structures formed. For example, a 0.005 inch layer of DuPont "Pyralin" Type 5081 polyimide (15.2 percent gravimetric solids, 50-70 poises viscosity) will be sufficient to prevent chemical and/or physical interaction between an alloy such as 4 percent Bismuth, 55.5 percent Lead, 40.5 percent Tin (commercially available as Cerro 400-1 alloy) and a plasma-deposited material such as beryllium. To improve the adhesion of plasma deposited materials on a polyimide coated mandrel, the cured polyimide coating can be given a moderate grit blast to roughen the surface. A moderate roughening of the surface may be described as one of 120-200 micro inch RMS surface roughness.

The fully cured dual coated mandrel is then ready for use in casting or plasma-deposition application. Once the selected material is deposited on the mandrel by conventional techniques to produce the desired structure, the unit is placed in a heated environment where the temperature is elevated above the melting point of the alloy undercoat. The liquid state alloy then flows from the unit leaving a space between the mandrel and the film adhering structure thereby allowing the mandrel to be easily withdrawn. The neutral type polyimide film can then be peeled from the structure leaving a free standing body.

The following examples will serve to illustrate the mandreling technique according to this invention:

#### EXAMPLE I

5 An aluminum base mandrel as shown in the drawing was coated with a 4 percent Bismuth, 55.5 percent Lead, 40.5 percent Tin alloy (commercially available as Cerro Type 400-1 alloy) having a melting point range of 170°C. to 198°C. The coated mandrel was machine finished leaving a smooth alloy layer of about 1/4 inch thick on the aluminum base. The surface of the coated mandrel was overcoated with a DuPont "Pyralin" Type 5081 polyimide precursor solution, 15.2 percent Gravimetric Solids, 50-70 poises viscosity, (commercially available as DuPont Pyralin 5081 polyimide) using an air brush spraying technique. A layer of approximately 0.001 inch thick was applied and then the N-Methyl Pyrrolidone and xylene solvent in the coating was extracted by oven heating the coated mandrel to approximately 125°C. for 15 minutes. This procedure was repeated until a 0.004 inch layer was built up whereupon the coated mandrel was cured at an elevated temperature of 150°C. for 16 hours.

20 The coated cured mandrel was then given a light grit blast of aluminum oxide to roughen the surface thereof so as to provide a better adhering surface for a plasma deposition of beryllium.

25 The roughened surface coated mandrel as shown in the drawing was plasma-sprayed with beryllium using the following:

|                        |                                                      |
|------------------------|------------------------------------------------------|
| Powder Lot             | Beryllium (commercially available as Brush V-1684-P) |
| Powder Size            | 325 Tyler mesh size and finer                        |
| Non-transfer-Arc Torch | Union Carbide's AT9 model                            |
| Electrode Gas          | 60 CFH Argon                                         |
| Powder Carrier Gas     | 80 CFH Argon and 40 CFH Argon + 15% Hydrogen         |
| Shield                 | Not used                                             |
| Current                | 195 amps.                                            |
| Voltage                | 58 volts                                             |
| Torch Pressure         | 31 PSIG                                              |
| Dispenser Pressure     | 36 PSIG                                              |
| Coating Time           | 9 minutes                                            |
| Coating Thickness      | 0.035" - 0.045"                                      |
| Torch Standoff         | 1 inch to 1 1/4 inches                               |
| Powder Feed Rate       | 13 grams per minute                                  |

40 After the plasma deposition of beryllium, the coated mandrel was placed in an oven and heated to 210°C. whereupon the Cerro Alloy melted and flowed from between the base mandrel and the polyimide film-coated beryllium structure leaving a space which enabled the mandrel to be easily removed. The polyimide film was then peeled from the structure leaving a free standing beryllium body having a contour identical to the mandrel shown in the drawing.

#### EXAMPLE II

45 A 13 UNC threaded rod, measuring  $1/2$  inch in diameter and 24 inches long, was coated with a 1.0 inch layer of Cerro Alloy 400-1 as in Example I, for a length of 19 inches. The surface of the Cerro layer was machined to a smooth finish yielding a final rod diameter of 1.92 inches. The smooth surface was then coated with a 0.005 inch multilayer of DuPont Pyralin 5081 polyimide precursor solution, as described in Example I, and followed thereafter by a light vapor blast of aluminum oxide to roughen the surface so as to make the surface amenable for a plasma-deposition of beryllium.

The polyimide coated surface was plasma-sprayed with beryllium using the following:

|                    |                                                           |    |
|--------------------|-----------------------------------------------------------|----|
| Powder Lot         | Beryllium powder (commercially available as Brush V-2484) | 5  |
| Powder Size        | 325 Tyler Mesh size and finer                             |    |
| Arc Torch          | Union Carbide's Model AT9                                 |    |
| Electrode Gas      | 60 CFH Argon                                              |    |
| Powder Carrier Gas | 80 CFH Argon and 40 CFH Argon + 15% Hydrogen              |    |
| Shield Current     | Not used                                                  | 10 |
| Voltage            | 180-200 amps.                                             |    |
| Torch Pressure     | 58-62 volts                                               |    |
| Dispenser Pressure | 32-35 PSIG                                                |    |
| Coating Time       | 37-39 PSIG                                                |    |
| Coating Thickness  | 60 minutes                                                |    |
| Torch Standoff     | .179 inch                                                 | 15 |
| Powder Feed Rate   | 1 1/4 inches                                              |    |
|                    | 12.8 grams per minute                                     |    |

After the plasma deposition of beryllium, the coated mandrel was placed in an oven and heated to 210°C. whereupon the Cerro Alloy melted and flowed from between the base mandrel and the polyimide film-coated beryllium structure leaving a space which enabled the mandrel to be easily removed. The polyimide film was then peeled from the structure leaving a free standing beryllium body having a contour identical to the machined Cerro Alloy coated mandrel.

What is claimed is:

1. a process for fabricating reusable mandrels designed for use in producing free-standing bodies comprising the steps:

- preparing a base mandrel of a material having a melting temperature above at least 650°C and substantially conforming in shape to a desired body to be deposited thereon and being dimensionally different than said body by a radial distance sufficient to allow for a dual coating build up on said mandrel(,), said body having zero draft angles or re-entrant geometries;
- depositing a metallic alloy on the surface of the mandrel to substantially conform to the shape of

said mandrel, said alloy having a melting temperature below 700°C and lower than the melting temperature of said base mandrel and said base mandrel material being substantially nonreactive with said metallic alloy; and

c. depositing and then curing at least one polyimide layer on said alloy deposited base mandrel to produce an overall coating that substantially conforms to the shape of the alloy coated base mandrel and that will essentially prevent any reaction between said alloy layer and the material of the body to be deposited thereon, said polyimide layer having a higher melting point than said alloy and being non-reactive with and easily separable from the material of the body to be deposited.

2. The process as in claim 1 wherein said base mandrel is selected from at least one of the group consisting of aluminum, brass, steel and copper.

3. The process as in claim 2 wherein said metallic alloy is selected from (at least one of the groups consisting of) an alloy from the group consisting of alloys of bismuth, lead, tin, cadmium, indium and antimony.

4. The process as in claim 3 wherein after step a) the following step is added:

b. machining said alloy deposited base mandrel to conform to the contour of a body to be produced thereon.

5. The process of claim 3 wherein said metallic alloy has a melting temperature below about 700°C. and a thickness between about 1/16 inch and 1 inch.

6. The process of claim 3 wherein said polyimide coated layer is between about 0.002 and about 0.010 inch thick.

7. The process of claim 6 (wherein said mandrel is for use in producing plasma-sprayed beryllium bodies) wherein beryllium is plasma-sprayed on said polyimide coated layer.

\* \* \* \* \*

UNITED STATES PATENT OFFICE  
CERTIFICATE OF CORRECTION

Patent No. 3,864,150 Issue Date February 4, 1975

Inventor(s) R. J. Baird and T. G. Everett, Jr.

It is certified that error appears in the above-identified patent  
and that said Letters Patent are hereby corrected as shown below:

Column 4, line 10; "174" should be -- 1/4 --

Column 5, line 36; "(;)" should be deleted.

Column 6, line 21; "(at least one of the groups consisting  
of)" should be deleted.

Column 6, line 35; "(wherein said mandrel is for use in  
producing plasma-sprayed beryllium  
bodies)" should be deleted.

Signed and Sealed this  
fourth Day of November 1975

[SEAL]

Attest:

RUTH C. MASON  
Attesting Officer

C. MARSHALL DANN  
Commissioner of Patents and Trademarks